

## 1

3,163,565

**PROCESS FOR PRODUCING A TOUGH STEEL  
FOR LOW TEMPERATURES**

Kamekichi Wada, Yawata, Japan, assignor to Yawata Iron & Steel Co., Ltd., Tokyo, Japan, a corporation of Japan

No Drawing. Filed June 19, 1962, Ser. No. 203,444  
Claims priority, application Japan, June 22, 1961,  
36/22,237

4 Claims. (Cl. 148—143)

This invention relates to the process for producing steel having high weldability and toughness at low temperatures. More particularly the present invention relates to a process for producing tough steel for low temperature service which contains no costly nickel and is easy to produce, simple to heat-treat and low in cost.

Generally, a steel has a transition temperature which is determined by its constituency and will absorb high energy at the time of breaking on the higher side of the transition temperature and low energy on the low temperature side. Therefore, it is considered necessary that a steel to be used at low temperatures should have a transition temperature low enough for the conditions which it is to be used under and further, should be tough.

A steel which has been extensively used for this purpose contains more than 2.5% nickel in order to keep the transition temperature low. However, when the alloying element nickel is added, the steel becomes costly and, further, special consideration is required for refining, ingotting, heating and rolling in the production of the steel and therefore the production cost is high.

The object of the present invention is to eliminate the aforementioned defects and to provide low-temperature tough steel which is easy to heat-treat and is low in cost.

A steel according to the present invention can easily be made by melting in an open-hearth furnace, electric furnace or pure oxygen converter. Its chemical composition is approximately less than 0.14% carbon, less than 0.5% silicon, 1.0 to 1.5% manganese, 0.01 to 0.04% aluminum and 0.008 to 0.020% nitrogen, less than 0.20% of one or more of the elements niobium, tantalum and vanadium if required with the remainder being iron and unavoidable impurities. Small amounts of some special element may be added when required. Steel having such a composition is produced by first melting, then rolling or forging, then heating to a temperature above 880° C., then quenching, further reheating to 600 to 700° C. and then cooling by air or the like.

Thus, the first of the fundamental features of the present invention is that when the aluminum and nitrogen are in a solid solution and supercooled in the steel they are deposited as aluminum nitride by heating from 600 to 700° C., which is below the A<sub>1</sub> transformation point, and then cooling so that the toughness at low temperatures may be improved. As already known, it is possible to improve the toughness by depositing aluminum nitride near the A<sub>3</sub> transformation point. However, the method of increasing the toughness by depositing aluminum nitride below the A<sub>1</sub> transformation point, as in the present invention, is far more effective than any known conventional method. The present invention is the first to discover and apply such fact. When the above mentioned heating temperature is below 600° C., the deposition of aluminum nitride will be volumetrically insufficient. When it is above 700° C., the structure will become austenite and the structure and deposited state will be non-uniform and undesirable.

## 2

The second of the features is to produce a steel having a fine ferrite structure. That is, said aluminum nitride will be highly effective when it is deposited in ferrite. Therefore, the steel is rapidly cooled from above 880° C. so that the steel will not have so-called hardened structure such as martensite or bainite but rather, should have a ferrite structure and that, before treating to deposit the aluminum nitride both the nitrogen and aluminum should be in solid solution in the steel.

- 10 In order that the aluminum and nitrogen are well liberated, the thermal condition before the depositing treatment must be restricted. The heating temperature above 880° C. in the heat-treatment of the steel according to the present invention is determined therefore. It is preferable that the heating time is as short as possible. However, as described later, the heating temperature must be kept in such range as will not make the crystal grain size coarse. The heating temperature before cooling is recommended to be about 880 to 950° C.
- 20 The cooling rate should be so rapid that no aluminum nitride will be deposited during cooling and must be controlled so that fine ferrite will appear and no hardened structure is made. A cooling rate of about 5 to 50° C./sec. is recommended. Further, in order to prevent aluminum nitride from being deposited, the cooling should be continued until a temperature below 600° C. is reached.

The limitation in the weight percentage of the elements contained in the steel of the present invention is explained below.

The range of aluminum in the steel is from 0.01 to 0.04% by weight and the range of nitrogen is from 0.008 to 0.020% by weight so that aluminum nitride is deposited below the A<sub>1</sub> transformation point. The carbon content is below 0.14% by weight so that a ferrite structure is obtained at the time of rapid cooling.

The silicon content is below 0.5% by weight which is the normal requirement in steel making. The manganese content is as high as is possible and is about 1.0 to 1.5% by weight so that, as already known, the toughness at low temperatures is increased and the weldability is improved.

Further, if necessary, there may be added a small amount, e.g., less than 0.2% by weight of one or more of the elements niobium, tantalum and vanadium each of which will form a fine carbide, stable even at high temperatures, and will reduce the hardenability, accelerate the production of fine ferrite and, at the same time, improve the weldability of the steel.

**EXAMPLE**

A steel containing the ingredients shown in Table 1 was produced by heating in an electric furnace to a temperature of 930° C. in 20 minutes. The steel was then rapidly cooled at a rate of 15° C./sec., then heated to a temperature of 625° C. for 30 minutes and was then cooled in air.

Table 1.—Examples of Chemical Compositions in Percent

| Sample signs | C   | Si  | Mn   | Al   | N    | Nb    | V     | Ta    |
|--------------|-----|-----|------|------|------|-------|-------|-------|
| A-----       | .08 | .22 | 1.12 | .018 | .009 | ----- | ----- | ----- |
| B-----       | .09 | .21 | 1.06 | .020 | .014 | ----- | ----- | ----- |
| C-----       | .08 | .23 | 1.15 | .029 | .012 | ----- | .02   | ----- |
| D-----       | .07 | .25 | 1.10 | .036 | .016 | ----- | .05   | ----- |
| E-----       | .10 | .22 | 1.09 | .026 | .010 | .03   | ----- | .02   |
| F-----       | .06 | .27 | 1.17 | .025 | .012 | .07   | ----- | ----- |

3  
*Table 2.—Examples of Mechanical Properties*

[As heated to 930° C. for 20 minutes, rapidly cooled, then heated to 625° C. for 30 minutes and cooled in air]

| Sample signs | Yielding point in kg./mm. <sup>2</sup> | Tensile strength kg./mm. <sup>2</sup> | Elongation in percent/200 mm. | Press notch Charpy broken surface transition temperature in ° C. |
|--------------|----------------------------------------|---------------------------------------|-------------------------------|------------------------------------------------------------------|
| A.....       | 36.8                                   | 48.3                                  | 27.2                          | -57                                                              |
| B.....       | 36.2                                   | 47.7                                  | 26.0                          | -61                                                              |
| C.....       | 41.4                                   | 51.1                                  | 27.5                          | -77                                                              |
| D.....       | 46.3                                   | 54.2                                  | 26.8                          | -80                                                              |
| E.....       | 40.0                                   | 51.4                                  | 26.3                          | -81                                                              |
| F.....       | 44.7                                   | 53.3                                  | 28.1                          | -85                                                              |

4  
*Table 3.—Examples of Deposition of Aluminum Nitride in Weight Percent by Heat-Treatment*

| Acid-soluble aluminum | Total nitrogen | Nitrogen as aluminum nitride |                                                                  |                                                                   |                                                                                                                         |
|-----------------------|----------------|------------------------------|------------------------------------------------------------------|-------------------------------------------------------------------|-------------------------------------------------------------------------------------------------------------------------|
|                       |                | Sample 1 (as rolled only)    | Sample 2 (as heated to 625° C. for 30 minutes and cooled in air) | Sample 3 (as heated to 930° C. for 20 minutes and rapidly cooled) | Sample 4 (as heated to 930° C. for 20 minutes, rapidly cooled, then heated to 625° C. for 30 minutes and cooled in air) |
| 0.020                 | 0.014          | 0.0002                       | 0.0112                                                           | 0.0004                                                            | 0.0123                                                                                                                  |

5  
*Table 4.—Examples of the Relation Between the Content of Nitrogen as Aluminum Nitride and Press Notch Charpy Transition Temperature*

[With the composition of Sample D in Table 1]

(a) In the table below the sample as rolled was heated to 625° C. for 30 minutes and was cooled in air. Ferrite-grain size No. 7-9 (A.S.T.M.).

|                                                                      |        |        |        |        |
|----------------------------------------------------------------------|--------|--------|--------|--------|
| Content of nitrogen in weight percent as aluminum nitride.....       | 0.0029 | 0.0051 | 0.0079 | 0.0144 |
| Press notch Charpy broken surface transition temperature in ° C..... | -18    | -21    | -38    | -42    |

(b) In the table below the steel was heated to 930° C. for 20 minutes, rapidly cooled, then heated to 625° C. for 30 minutes and cooled in air. Ferrite-grain size No. 9-11 (A.S.T.M.).

|                                                                |        |        |        |        |
|----------------------------------------------------------------|--------|--------|--------|--------|
| Content of nitrogen in weight percent as aluminum nitride..... | 0.0031 | 0.0054 | 0.0083 | 0.0152 |
| Press notch Charpy fracture transition temperature in ° C..... | -28    | -34    | -61    | -58    |

As is apparent from the press notch Charpy transition temperature in Table 2, the steel according to the present invention showed a favorable toughness at low temperatures. This was realized only by the combination of the above mentioned two fundamental features.

The deposition of aluminum nitride by heat-treatment shall be described now.

In Table 3, sample 1 is as rolled, sample 2 is the same as sample 1 except it was heated to 625° C. for 30 minutes and then cooled in air, sample 3 is the same as sample 1 except it was heated to 930° C. for 20 minutes and then rapidly cooled and sample 4 is the same as sample 3 except it was heated to 625° C. for 30 minutes and then cooled in air. In (a) and (b) in Table 4 there is shown the relationship between the amount of aluminum nitride and the press notch Charpy broken surface transition temperature on the rolled sample and the sample heated to 930° C. for 20 minutes and rapidly cooled, both of which were heated to 625° C. for 30 minutes and then cooled in air for the depositing treatment. In both the rolled sample and the rapidly cooled sample, after the depositing treatment, aluminum nitride was greatly deposited and an increase in low-temperature toughness was

observed. However, it is clearly seen that the sample which was rapidly cooled had better values than the rolled sample which is explained by the fact that there is a difference in the ferrite grain size between the two samples which is caused by the heating of the one sample to a temperature of 930° C. for 20 minutes and then rapidly cooling said sample.

What I claim is:

1. A process for producing a tough steel for low temperature service comprising heating a low carbon steel containing 0.01 to 0.04 weight percent aluminum, 0.008 to 0.02 weight percent nitrogen and less than 0.14 weight percent carbon to a temperature above the A<sub>3</sub> transformation point, quickly cooling said steel at a cooling rate of 5 to 50 degrees centigrade per second to a tempera-

ture below 600° C. whereby there is produced a fine ferrite structure in said steel and the liberated aluminum and nitrogen are in solid solution; reheating the cooled steel to a temperature of about 600 to 700° C. and cooling the steel whereby the aluminum and nitrogen are deposited in said steel as aluminum nitride.

2. A process for producing a tough steel for low temperature service comprising heating a low carbon steel containing 0.01 to 0.04 weight percent aluminum, 0.008 to 0.02 weight percent nitrogen, less than 0.50% silicon and less than 0.14 weight percent carbon to a temperature of about 880 to 950° C., quickly cooling said steel at a cooling rate of from 5 to 50 degrees centigrade per second to a temperature below 600° C. whereby there is produced a fine ferrite structure in said steel and the liberated aluminum and nitrogen are in solid solution; reheating the cooled steel to a temperature of about 600 to 700° C. and cooling the steel to room temperature whereby the aluminum and nitrogen are deposited in said steel as aluminum nitride.

3. A process for producing a tough steel for low temperature service comprising heating a steel containing 1.0 to 1.5 weight percent manganese, 0.01 to 0.04 weight percent aluminum, 0.008 to 0.20 weight percent nitrogen, less than 0.14 weight percent carbon, less than 0.50 weight percent silicon with the remainder being iron and incidental impurities to a temperature of about 880 to 950° C. and quickly cooling said steel at a cooling rate of from 5 to 50 degrees centigrade per second to a temperature below 600° C. whereby there is produced a fine ferrite structure in said steel and the liberated aluminum and nitrogen are in solid solution; reheating the cooled steel to a temperature of about 600 to 700° C. and cooling the steel to room temperature whereby the aluminum and nitrogen are deposited in said steel as aluminum nitride.

4. A process for producing a tough steel for low temperature service comprising heating a steel containing 1.0 to 1.5 weight percent manganese, 0.01 to 0.04 weight percent aluminum, 0.008 to 0.20 weight percent nitrogen, less than 0.14 weight percent carbon, less than 0.50 weight percent silicon and at least one alloying element selected from the group consisting of niobium, tantalum and vanadium, the total amount of said alloying elements

being less than 0.20 weight percent with the remainder being iron and incidental impurities to a temperature of about 880 to 950° C. and quickly cooling said steel at a cooling rate of from 5 to 50 degrees centigrade per second to a temperature below 600° C. whereby there is produced a fine ferrite structure in said steel and the liberated aluminum and nitrogen are in solid solution; reheating the cooled steel to a temperature of about 600 to 700° C. and cooling the steel to room temperature whereby the aluminum and nitrogen are deposited in said steel as aluminum nitride.

## References Cited by the Examiner

## UNITED STATES PATENTS

3,028,270 4/62 Morita et al. ----- 148—143

## FOREIGN PATENTS

5 786,993 11/57 Great Britain.

808,556 2/59 Great Britain.

DAVID L. RECK, Primary Examiner.

10 RAY K. WINDHAM, Examiner.